# EUROPEAN PATENT SPECIFICATION

(11) **EP 2 634 310 B1**
(45) Date of publication and mention of the grant of the patent: **26.11.2014**
(21) Application number: 13157139.0
(22) Date of filing: 28.02.2013
(51) Int. Cl.: D21H 21/44

(54) **Security Paper that is Detectable by Metal Detectors**
Von Metalldetektoren erfassbares Sicherheitspapier
Papier de sécurité détectable par des détecteurs de métaux

(30) Priority: 28.02.2012 KR 20120020399
(43) Date of publication of application: 04.09.2013
(73) Proprietor: Samsung Electronics Co., Ltd, Gyeonggi-do 443-742 (KR)
(72) Inventor: Jung, Taek-yong, Gyeonggi-do (KR); Jung, Chang-woo, Seoul (KR); Choi, Ae-kyung, Gyeongsangbuk-do (KR)
(74) Representative: Russell, Tim

(56) References cited:
- EP-A2- 0 374 930
- WO-A1-99/28852
- WO-A1-2004/043706
- GB-A- 546 333
- US-A- 3 053 676
- US-A- 5 004 643
- US-A1- 2009 017 334

## Description

The present invention relates to a security paper, and in particular, to a security paper that is detectable by a metal detector.

The increased significance of preventing leakage of information has lead to the development of security technologies for blocking the leakage of various data recording media. However, in the case of a recording media, such as paper, it is difficult to control transferring of the recording media. Accordingly, research into security paper that enables the transferring of paper to be blocked is performed in various fields.

To effectively manage documents, printer manufacturers have been providing a program for managing printing situations together with a printer, since the 1990s. Also, recently, many businesses have adopted management of printing system (MPS). Furthermore, printer manufacturers and printer users consider using security paper together with MPS.

As a method of manufacturing security paper, various methods, for example, a method of manufacturing security paper using a hidden line, a method of manufacturing security paper using a fluorescent material, or a method of manufacturing security paper using a metallic tag, are known. Also, for use of metal detectors which are widely used in security systems, manufacturing of security paper that is detectable by a metal detector is taken into consideration.

Metal detectors are used to detect the presence of a metallic material even when the metallic material is not in sight, by using electromagnetic induction and eddy current. When a magnetic field occurs in a coil in which an alternative current flows, eddy current occurs in a metal due to the magnetic field. The eddy current that occurs in the metal causes a magnetic field, which is detected by metal detectors to confirm presence of the metal. As well known, metal detectors are used for various purposes, such as removing of mines, detecting of arms at airport security check points, archaeological digging, treasure hunting, geological prospecting, and detecting of foreign materials in food.

Various papers having a stack structure including a metal layer have been disclosed. For example, KR 10-2008-0107977 discloses a printing paper for security purposes, including first and second paper sheets having surfaces attached to each other by using an adhesive material; and at least one detection tag interposed between the attached surfaces of the first and second paper sheets. Also, according to the disclosure of the above-described reference, the detection tag may include an amorphous soft alloy, a metal thin film may be further formed between the attached surfaces of the first and second paper sheets, and the first paper sheet or the second paper sheet may have a surface on which metal may be vacuum-deposited or transferred.

US 2009/0017334 describes a recoding paper having a magnetic material-containing layer, that includes a magnetic material that generates a large Barkhausen effect and a filler, and is disposed between pulp layers containing a pulp.

US 5,004,643 describes a process for treating a porous web (especially fabric) to produce a novel silicone polymer internally coated web. In the process, a starting curable liquid silicone polymer is coated under pressure upon one surface of the web.

GB 546,333 describes a metallic coated sheet material simulating metal foil. The coated sheet has a luminous apparent relectance of less than 0.2, an apparatus reflectance contrast value of at least 25, and an emissivity value of not more than 0.2.

However, laminating of many layers may cause many problems: for example, manufacturing costs may be increased; curling of paper may occur during the laminating process; and excess volatile organic compounds (VOCs) may be included in paper due to an adhesive used during the laminating process.

VOCs contained in paper may be released by heating during printing. The amount of VOCs released during printing is restricted according to an international standard due to environmental issues. Accordingly, if VOCs are released in great amounts from paper, it would be disadvantageous. In particular, when a laser printer is used, the temperature during the fixing process is, for example, from about 120°C to about 200°C. Accordingly, the amount of released VOCs may be very high.

As disclosed in Korean Patent No. 10-2008-0107977, when a metal tag is used, a black ink layer for shielding a tag may be additionally needed. When a paper sheet contains a black ink layer, paper brightness may be lowered. Brightness is one of the important factors when a quality of paper is taken into consideration. When the paper brightness is lowered, the quality of an image printed on paper is lowered.

According to a first aspect of the present invention, there is provided a security paper which includes a substrate sheet; and a detectable layer that is attached to at least a portion of at least a surface of the substrate sheet, wherein the detectable layer comprises metal powder, a silicon-containing compound, and a water-soluble binder resin.

A security paper according to the present invention may have high brightness and a low volatile organic compounds (VOC) content and be detectable by a metal detector.

The security paper may further include an under-coating layer interposed between the substrate and the detectable layer.

According to a second aspect of the present invention, there is provided a composition for forming a detectable layer, the composition including: metal powder, a silicon-containing compound, a water-soluble binder resin, and water.

According to a third aspect of the present invention, there is provided a method of producing a security paper including: coating the composition according to the invention in its second aspect on at least a portion of at least a surface of a substrate; and drying the coated composition.

The method may further include, prior to the coating of the composition, forming an under-coating layer on the substrate.

Embodiments will now be described more fully with reference to the accompanying drawings, in which exemplary embodiments are shown. Expressions such as "at least one of," when preceding a list of elements, modify the entire list of elements and do not modify the individual elements of the list.

A security paper according to the present invention includes a substrate sheet, and a detectable layer that is attached to at least a portion of at least a surface of the substrate, wherein the detectable layer includes metal powder, a silicon-containing compound, and a water-soluble binder resin.

The substrate may be, for example, paper or a resin film. The paper may be, for example, a paper that is coated with a resin or a paper that is not coated with a resin. The paper that is not coated with a resin may be, for example, wood-free paper or thin paper. The paper that is coated with a resin may be, for example, art paper or coated paper, cast-coated paper, or resin-coated paper. The resin film may be, for example, polyethylenetelephthalate, polycarbonate, or cellulose acetate. The thickness of the substrate is not particularly limited.

The detectable layer may be attached to at least a portion of at least a surface of the substrate. The detectable layer may be coated along a complete surface of the substrate. The detectable layer may be coated on a portion of a surface of the substrate. A region for the detectable layer may be appropriately selected according to the detectability of the metal detector. Alternatively, to increase the detectability of the security paper, the detectable layer may be attached to a portion of each of both surfaces of the substrate: in this case, the detectable layer may be attached to a surface of the substrate and the other surface of the substrate; or the detectable layer may be attached to a surface of the substrate and a portion of the other surface of the substrate; or the detectable layer may be attached to a portion of a surface of the substrate and the other surface of the substrate; or the detectable layer may be attached to a portion of a surface of the substrate and a portion of the other surface of the substrate. When the detectable layer is located on a portion of any one of surfaces of the substrate, the location of the detectable layer is not limited. Accordingly, the detectable layer may be located in either a printing area or a non-printing area, or both a printing area and a non-printing area.

The detectable layer includes a metal powder, a silicon-containing compound and a binder resin.

When only metal powder is used, the detectability of the security paper is high. However, the manufacturing costs for security paper may increase, and it would be difficult to coat the detectable layer on the substrate. Accordingly, by using metal powder and a silicon-containing compound together, manufacturing costs for the security paper may decrease and the detectable layer may be easily coated on the substrate. Also, the security paper may have an excellent detectability.

The metal powder may be any one of metals that are detectable by a metal detector. Examples of the metal powder include iron, cobalt, nickel, manganese, silver, copper, zirconium, aluminium, and combinations thereof. For example, the metal powder may be a ferromagnetic metal. Examples of the ferromagnetic metal include iron, cobalt, nickel, manganese, and combinations thereof. Due to the use of ferromagnetic metal powders, excellent detectability may be obtained for relatively small amounts of the metal powder.

The particle size of the metal powder is not particularly limited. However, when the particle size of the metal powder is too small, the detectability may be lowered, and when the particle size of the metal powder is too great, dispersibility of the metal powder in a composition for forming the detectable layer may be lowered. For example, the average particle size of the metal powder may be in the range of about 0.1 µm to about 100 µm.

The detectable layer comprises a silicon-containing compound. The silicon-containing compound may be an organosilicon compound in which at least one carbon atom in an organic compound is substituted with a silicon atom, or the silicon-containing compound may be an inorganic silane.

Due to the use of a silicon-containing compound, the amount of metal powder may be reduced while the detectability of the security paper is maintained, and also, the stability of the coating solution may be increased.

Examples of suitable silicon-containing compounds include halogenosilanes, alkoxysilanes, aminosilanes, silane coupling agents, fluoroalkylsilanes, reactive siloxane oligomers, and combinations thereof.

Detailed examples of halogenosilanes are chlorosilane, trichlorosilane, methyldichlorosilane, and phenyldichlorosilane.

Detailed examples of alkoxysilanes are methyldiethoxysilane, methyldimethoxysilane, phenyldimethoxysilane, trimethoxysilane, and triethoxysilane.

Detailed examples of aminosilanes are methyldiaminosilane and triaminosilane.

Detailed examples of aminoxysilanes are methyldiaminoxysilane and triaminoxysilane.

Detailed examples of acyloxysilanes are methyldiacetoxysilane, phenyldiacetoxysilane, and triacetoxysilane.

The water-soluble binder resin may increase the stability of metal powder and the silicon-containing compound and the adhesion force thereof with respect to the substrate. The water-soluble binder resin may be, for example, polyvinylalcohol, polyvinylpyrrolidone, cellulose, polyacryl, polyester, latex, or a combination thereof.

When the detectable layer has too low a content of the metal powder, the detectability may be reduced. On the other hand, when the detectable layer has too high a content of the metal powder, the detect-ability of security paper may be increased, however the cost for materials used in preparing the security paper may be increased too much. Therefore, for example, the amount of the metal powder in the detectable layer may be in the range of about 1 wt% to about 10 wt% based on 100 wt% of the total weight of the detectable layer. However, even when the metal powder content is about 10 wt% or less, the security paper may have an excellent detectability. Such an effect may be due to the fact that the silicon-containing compound also has a detectability and the coating solution thereof has an excellent dispersibility, and thus, detectability of the security paper is also improved.

When the amount of the silicon-containing compound in the detectable layer is too low, the manufacturing costs may be increased and/or dispersibility of the coating solution thereof may be reduced. When the amount of the silicon-containing compound in the detectable layer is too great, the detectability may be reduced. For example, the amount of the silicon-containing compound in the detectable layer may be in the range of about 1 wt% to about 50 wt% based on 100 wt% of the total weight of the detectable layer. In general, the silicon-containing compound is relatively inexpensive compared to the metal powder. Accordingly, even when the amount of the silicon-containing compound is as high as about 50 wt% based on 100 wt% of the total weight of the detectable layer, the effects of the silicon-containing compound on the manufacturing costs for security paper may be negligible.

The amount of the water-soluble binder resin in the detectable layer may be the remainder after the weights of the metal powder and the silicon-containing compound are subtracted from the total weight of the detectable layer. For example, the amount of the water-soluble binder resin in the detectable layer may be in the range of about 50 wt% to about 95 wt% based on 100 wt% of the total weight of the detectable layer. Although the amount of the water-soluble binder resin is as low as about 50 wt%, the water-soluble binder resin may sufficiently function as providing an adhesion force between the detectable layer and the substrate and fixing the metal powder and the silicon-containing compound in the detectable layer.

When the thickness of the detectable layer increases, the detectability of the security paper may increase. However, when the detectable layer is too thick, when security paper is used in an inkjet printer, a decrease in ink adsorption force and a decrease in ink drying speed may occur, and when security paper is used in a laser printer, a decrease in fixability of toner and a decrease in transferring efficiency of toner may occur. Also, the greater thickness the detectable layer has, the higher manufacturing costs security paper has. When the detectable layer is too thin, detectability may decrease. For example, the thickness of the detectable layer may be in the range of about 1 µm to about 10 µm.

The detectable layer may have the same level of brightness as a typical duplicating paper. Brightness of paper is a critical factor in determining the quality of an image, and when the level of brightness decreases, chroma or brightness of a printed image may decrease.

The shape and area of the detectable layer of the security paper are not particularly limited. For example, even when three detectable layers each having a bar shape having a width of 1 mm extending from an upper portion to a lower portion of security paper are formed on a surface of security paper, excellent detectability was obtained.

According to an embodiment of the present invention, the security paper may further include an under-coating layer between the substrate and the detectable layer. The under-coating layer may enhance the adhesion force between the substrate and the detectable layer. When the adhesion force is weak, during printing using a printer, the substrate and the detectable layer may be exfoliated from each other. The under-coating layer is useful when the substrate is a resin film. The under-coating layer is more useful when the substrate is a hydrophobic resin film.

The under-coating layer may be, for example, an adhesive layer. Alternatively, to minimize the VOC content in the security paper, the under-coating layer may be formed of a water-soluble resin. A water-soluble resin for use in the under-coating layer may be, for example, a polyol-based resin, an acryl-based resin, a poly urethane-based resin, a vinyl resin, or a combination thereof.

The under-coating layer may further include an inorganic filler. An example of the inorganic filler may be, for example, calcium carbonate, titanium dioxide, clay, talc, silica, or alumina.

When the under-coating layer is too thick, in the case of an ink-jet printer, an ink adsorption force may be reduced, and in the case of a laser printer, fixability may be lowered. When the under-coating layer is too thin, the increase in the adhesion force between the substrate and the detectable layer may be negligible. For example,the thickness of the under-coating layer may be in the range of about 0.1 µm to about 5 µm.

The under-coating layer may be formed to overlap where at least the detectable layer is formed, for example.

Another aspect of the invention provides a composition for forming a detectable layer, wherein the composition includes metal powder, a silicon-containing compound, a water-soluble binder resin, and water.

Water functions as a solvent for the water-soluble binder resin, a solvent or a dispersing medium for the silicon-containing compound, and a dispersing medium for the metal powder. Due to the use of water and the water-soluble binder resin, the VOC content in the detectable layer of the security paper may be minimized.

The amount of water in the composition may be appropriately determined in such a way that the composition retains a viscosity that is appropriate for the coating method used in coating the composition on a substrate. When the water content in the composition is too low, dispersibility or coating properties may be reduced, and when the water content in the composition is too high, the thickness of the detectable layer may not be increased. For example, the water content in the composition may be in the range of about 100 parts by weight to about 1000 parts by weight based on 100 parts by weight of all of the components that form the detectable layer. For example, the viscosity of the composition may be in the range of about 100 cP to about 5000 cP.

To effectively disperse metal powder, the composition may further include a dispersing agent. The dispersing agent may be, for example, polycarboxylate, sodium polyphosphate, or a combination thereof. An amount of the dispersing agent may be, for example, in the range of about 0.5 parts by weight to about 10 parts by weight, based on 100 parts by weight of the metal powder.

Another aspect of the present invention provides a method of manufacturing security paper, the method including: coating the composition described above on at least a portion of at least a surface of a substrate; and drying the coated composition.

The substrate may be used in a form of, for example, a sheet or roll.

The coating may be performed by using various coating methods, for example, spraying, painting, or printing. For example, the coating may be performed by using a blade coater, a bar coater, a gravure coater, an air-knife coater, a roll-to-roll coater, or the like.

The drying may be performed by using a typical drying method, for example, natural drying, freeze-drying, or hot drying.

According to an embodiment, the method may further include, prior to the coating of the composition, forming an under-coating layer on the substrate.

The forming of the under-coating layer may be performed by coating a composition for forming an under-coating layer which includes an aqueous solution of a water-soluble resin on at least a portion of at least a surface of the substrate. Drying of the coated under-coating layer forming composition may be performed together with the drying of the composition for forming the detectable layer. Alternatively, the forming of the under-coating layer may be performed by coating the under-coating layer forming composition including an aqueous solution of a water-soluble resin on at least a portion of at least a surface of the substrate, followed by drying the coated under-coating layer forming composition. The coating and drying of the under-coating layer forming composition may be performed by using the same methods as described above with reference to the composition for forming the detectable layer. The water content of the under-coating layer forming composition may be appropriately selected to obtain a viscosity that is appropriate for a selected coating method. When the water content of the under-coating layer forming composition is too low, coating properties may decrease, and when the water content in the under-coating layer forming composition is too high, drying time may be too long. For example, the water content of the under-coating layer forming composition may be in the range of about 500 parts by weight to about 10000 parts by weight based on 100 parts by weight of the water-soluble binder resin. For example, the viscosity of the under-coating layer forming composition may be in the range of about 10 cP to about 1000 cP.

### Examples

### Example 1 --- Preparation of Composition for Forming Detectable Layer

18.0 parts by weight of polyvinylalcohol (a product of Korea OCI Company) 1.0 parts by weight of cobalt powder (a product of Korea Seochong Materials Company, having an average particle size of 5 µm), 1.0 parts by weight of a silane coupling agent (a product of Korea Siltech Company, TSL8311), 0.1 parts by weight of dispersing agent (a product of Jungwoo Chemistry-Korea, Kosant A-40), and 80.0 parts by weight of water were mixed by using a ball mill to prepare a composition for mixing a detectable layer.

### Example 2 --- Preparation of Composition for Forming Detectable Layer

15.3 parts by weight of hydroxypropylmethylcellulose (a product of Samsung Fine Chemicals - Korea, Anycoat-C), 1.0 parts by weight of cobalt powder (a product of Seochong Materials Company-Korea, having an average particle size of 10 µm), 1.0 parts by weight of a silane coupling agent (a product of Siltech Company-Korea, TSL8380), 0.1 parts by weight of dispersing agent (a product of Jungwoo Chemistry-Korea, Kosant TT-400), and 80.0 parts by weight of water were mixed by using a ball mill to prepare a composition for mixing a detectable layer.

### Example 3 --- Preparation of Composition for Forming Detectable Layer

18.0 parts by weight of polyvinylalcohol (a product of OCI Company-Korea, 1.0 parts by weight of zirconium powder (a product of Seochong Materials Company -Korea, having an average particle size of 5 µm), 1.0 parts by weight of an alkoxysilane (a product of Siltech Company - Korea, TSL8124), 0.1 parts by weight of dispersing agent (a product of JungwooChemistry-Korea, Kosant TT-400), and 80.0 parts by weight of water were mixed by using a ball mill to prepare a composition for mixing a detectable layer.

### Example 4 --- Preparation of Security Paper

The composition prepared according to Example 1 was coated completely on the surface of a sheet of wood-free paper having a size 80 g/m² manufactured by Hansol Paper Company by using a bar coater. The coated sheet was dried at a temperature of 100°C for 1 minute. A weight of the prepared security paper was 90 g/m², and a weight and a thickness of the formed detectable layer were 10 g/m² and 10 µm, respectively.

### Example 5 --- Preparation of Security Paper

The composition prepared according to Example 3 was coated completely on the surface of a sheet of wood-free paper having a size 80 g/m² manufactured by Hansol Paper Company by using a bar coater. The coated sheet was dried at a temperature of 100°C for 1 minute. A weight of the prepared security paper was 90 g/m², and a weight and a thickness of the formed detectable layer were 10 g/m² and 10 µm, respectively.

### Example 6 --- Preparation of Security Paper

The composition prepared according to Example 3 was coated completely on the surface of a sheet of wood-free paper having a size 80 g/m² manufactured by Hansol Paper Company by using a bar coater. The coated sheet was dried at a temperature of 100°C for 1 minute. A weight of the prepared security paper was 90 g/m², and a weight and a thickness of the formed detectable layer were 10 g/m² and 10 µm, respectively.

### Example 7 --- Preparation of Security Paper

The composition prepared according to Example 1 was coated completely on the surface of a sheet of wood-free paper having a size 80 g/m² manufactured by Hansol Paper Company by using a bar coater. The coated sheet was dried at a temperature of 100°C for 1 minute. A weight of the prepared security paper was 85 g/m², and a weight and a thickness of the formed detectable layer were 5 g/m² and 5 µm, respectively.

### Example 8 --- Preparation of Security Paper

Security paper was prepared in the same manner as in Example 4, except that 107 µm PET(SH62) manufactured by SKC Company was used as a substrate. A thickness of a formed detectable layer of the security paper was 10 µm.

### Comparative Example 1 --- Preparation of Security Paper

Security paper was prepared in the same manner as in Example 4, except that a weight of a formed detectable layer was 0.5 g/m² after drying. A thickness of the detectable layer of the security paper was 0.5 µm.

### Comparative Example 2 --- Preparation of Security Paper

Security paper was prepared in the same manner as in Example 4, except that a weight of a formed detectable layer was 12 g/m² after drying. A thickness of the detectable layer of the security paper was 12 µm.

### Comparative Example 3 --- Preparation of Commercially Available Security Paper

Security paper (10-2008-0108063, 10-2008-0107977) manufactured by Koreit Company, including a cobalt-based metal chip disposed between two sheets of paper, was purchased.

### Evaluation Results

Brightness, optical density of printed images, ink adsorption force, toner fixability, a TVOC release amount during printing, and a metal detector detect-ability of the security papers manufactured according to Examples 4 to 8 and Comparative Examples 1 to 3 were evaluated.
- Brightness: the brightness of the security paper was measured 10 times by using a colorimeter (USA "McBeth" Company "SpectroEye") and an average thereof was used. The higher brightness, the better.
- Optical density of printed images: a yellow block image was printed on the security paper by using a CLP-315 printer manufactured by Samsung Electronics Co., Ltd -Korea, and then the optical density of a yellow block image was measured by using a colorimeter (USA "McBeth" Company "SpectroEye"). The higher value, the more distinct the image.
- Ink adsorption force: a black block image was printed on the security paper by using Japan EPSON Company stylus 915 inkjet printer. 30 seconds after the printing, the black block image was scrubbed three times by using a pendulum having a weight of 100 g, and then, the bleeding level of the black block image was measured based on a 5-point method. The lower the bleeding level, the greater the ink adsorption force.
- Toner fixability: a black block image was printed on security paper by using a CLP-315 color laser printer manufactured by Samsung Electronics Co., Ltd -Korea, and then, first optical density was measured by using SpectroEye measuring device of USA McBeth Company. 60 seconds after, a 30M tape was attached to a black block image, and then a pendulum having a weight of 500g was scrubbed thereon ten times, and then, the tape was removed and a second optical density of the black block image was measured. The ratio of the first optical density to the second optical density is the residual rate. The higher the residual rate, the higher the toner fixability.
- TVOC release amount during printing: The TVOC release amount was measured according to the guideline "Blue Angel" presented by a German material test research center (BAM) (printer: a mono laser printer SCX-6545N manufactured by Samsung Electronics Co., Ltd -Korea, the test method: RAL-UZ 122).
- Metal detector detect-ability: whether the security paper was detectable by a metal detector (USA Dokscom Company AD-2600S) was confirmed. The test results were evaluated as "detection" or "non-detection." The distance between the metal detector and the security paper was 5 cm.

Evaluation results obtained by using the security papers of Examples 4 to 8 and Comparative Examples 1 to 3 in the above tests are shown in Table 1.

**Table 1**

| | Brightness (%) | Printed image optical density | Ink absorption force | Toner fixability (%) | TVOC (mg/h) | Detectability |
|---|---|---|---|---|---|---|
| Example 4 | 90 | 1.25 | 1 | 95 | 9 | Detection |
| Example 5 | 88 | 1.21 | 1 | 93 | 8 | Detection |
| Example 6 | 90 | 1.23 | 1 | 94 | 10 | Detection |
| Example 7 | 91 | 1.27 | 1 | 95 | 8 | Detection |
| Example 8 | 90 | 1.23 | 2 | 88 | 10 | Detection |
| Comparative Example 1 | 90 | 1.23 | 1 | 92 | 7 | Non-detection |
| Comparative Example 2 | 89 | 1.22 | 3 | 80 | 10 | Detection |
| Comparative Example 3 | 80 | 1.05 | 1 | 85 | 21 | Detection |

The security paper of Examples 4 to 8 had a brightness of 88% to 91% and the security paper of Comparative Example 3 had a brightness of 80%. That is, the security paper of Examples 4 to 8 had a brightness 10% greater than that of the security paper of Comparative Example 3.

Images printed on the security paper of Examples 4 to 8 had an optical density of 1.21 to 1.27, and an image printed on the security paper of Comparative Example 3 had an optical density of 1.05. That is, images printed on the security paper of Examples 4 to 8 had an optical density 15% greater than that of an image printed on the security paper of Comparative Example 3.

The security paper of Examples 4 to 7 had a toner fixability of 93% to 95% and the security paper of Comparative Example 3 had a toner fixability of 85%. That is, the security paper of Examples 4 to 7 had a toner fixability 9% greater than that of the security paper of Comparative Example 3.

The security paper of Examples 4 to 78 had a TVOC release amount of 8 to 10 mg/h and the security paper of Comparative Example 3 had a TVOC release amount of 21 mg/h. That is, the security paper of Examples 4 to 8 had a TVOC release amount 52% greater than that of the security paper of Comparative Example 3.

As described above, the security paper of Examples 4 to 8 has excellent detectability with respect to a metal detector as well as excellent printing qualities.

The security paper according to the present invention is detectable by a metal detector. The security paper has high brightness. Accordingly, an image printed on the security paper has excellent qualities. Also, the security paper has a low volatile organic compound (VOC) content.

While the present invention has been described in connection with certain exemplary embodiments thereof, it is to be understood that the invention is not limited to the disclosed embodiments, but, on the contrary, is intended to cover various modifications and equivalent arrangements included within the scope of the appended claims.

## Claims

1. A security paper comprising:
a substrate; and
a detectable layer that is attached to at least a portion of at least a surface of the substrate,
wherein the detectable layer comprises metal powder, a silicon-containing compound, and a water-soluble binder resin.

2. The security paper of claim 1, wherein the substrate is a paper that is coated with a resin, a paper that is not coated with a resin, or a resin film.

3. The security paper of claim 1 or claim 2, wherein the metal powder of the detectable layer is selected from the group consisting of iron, cobalt, nickel, manganese, and combinations thereof.

4. The security paper of any preceding claim, wherein the average particle size of the metal powder is in the range of 0.1 µm to 100 µm.

5. The security paper of any preceding claim, wherein the silicon-containing compound of the detectable layer is selected from the group consisting of halogenosilanes, alkoxysilanes, aminosilanes, silane coupling agents, fluoroalkylsilanes, reactive siloxane oligomers, and combinations thereof.

6. The security paper of any preceding claim, wherein the water-soluble binder resin of the detectable layer is selected from the group consisting of polyvinylalcohol, polyvinylpyrrolidone, polyacrylate, polyester, latex, and combinations thereof.

7. The security paper of any preceding claim, wherein the amount of the metal powder in the detectable layer is in the range of 1 wt% to 10 wt% based on 100 wt% of the total weight of the detectable layer.

8. The security paper of any preceding claim, wherein the amount of the silicon-containing compound in the detectable layer is in the range of 1 wt% to 50 wt% based on 100 wt% of the total weight of the detectable layer.

9. The security paper of any preceding claim 1, wherein the thickness of the detectable layer is in the range of 1 µm to 10 µm.

10. The security paper of any preceding claim, further comprising an under-coating layer interposed between the substrate and the detectable layer.

11. The security paper of claim 10, wherein the under-coating layer comprises a water-soluble resin.

12. The security paper of claim 10 or claim 11, wherein the thickness of the under-coating layer is in the range of 0.1 µm to 5 µm.

13. A composition for forming a detectable layer, the composition comprising: metal powder, a silicon-containing compound, a water-soluble binder resin, and water.

14. The composition of claim 13, wherein the composition further comprises a dispersing agent.

15. A method of producing a security paper, the method comprising:
coating the composition according to any one of claims 13 and 14 on at least a portion of at least a surface of a substrate; and
drying the coated composition.

## Patentansprüche

1. Sicherheitspapier, Folgendes umfassend:
ein Substrat und
eine erkennbare Schicht, die an mindestens einem Abschnitt mindestens einer Oberfläche des Substrats angebracht ist,
wobei die erkennbare Schicht Metallpulver, eine siliciumhaltige Verbindung und ein wasserlösliches Bindemittelharz umfasst.

2. Sicherheitspapier nach Anspruch 1, wobei das Substrat ein Papier ist, das mit einem Harz beschichtet ist, ein Papier, das nicht mit einem Harz beschichtet ist, oder eine Harzfolie.

3. Sicherheitspapier nach Anspruch 1 oder Anspruch 2, wobei das Metallpulver der erkennbaren Schicht aus der Gruppe ausgewählt ist, die aus Eisen, Kobalt, Nickel, Mangan und Kombinationen daraus besteht.

4. Sicherheitspapier nach einem der vorhergehenden Ansprüche, wobei die durchschnittliche Partikelgröße des Metallpulvers im Bereich von 0,1 µm bis 100 µm liegt.

5. Sicherheitspapier nach einem der vorhergehenden Ansprüche, wobei die siliciumhaltige Verbindung der erkennbaren Schicht aus der Gruppe ausgewählt ist, die aus Halogensilanen, Alkoxysilanen, Aminosilanen, Silan-Kopplungsmitteln, Fluoralkylsilanen, reaktiven Siloxanoligomeren und Kombinationen daraus besteht.

6. Sicherheitspapier nach einem der vorhergehenden Ansprüche, wobei das wasserlösliche Bindemittelharz der erkennbaren Schicht aus der Gruppe ausgewählt ist, die aus Polyvinylalkohol, Polyvinylpyrrolidon, Polyacrylat, Polyester, Latex und Kombinationen daraus besteht.

7. Sicherheitspapier nach einem der vorhergehenden Ansprüche, wobei die Menge des Metallpulvers in der erkennbaren Schicht, bezogen auf 100 Gew.-% der Gesamtmenge der erkennbaren Schicht, im Bereich von 1 Gew.-% bis 10 Gew.-% liegt.

8. Sicherheitspapier nach einem der vorhergehenden Ansprüche, wobei die Menge der siliciumhaltigen Verbindung in der erkennbaren Schicht, bezogen auf 100 Gew.-% der Gesamtmenge der erkennbaren Schicht, im Bereich von 1 Gew.-% bis 50 Gew.-% liegt.

9. Sicherheitspapier nach einem der vorhergehenden Ansprüche, wobei die Dicke der erkennbaren Schicht im Bereich von 1 µm bis 10 µm liegt.

10. Sicherheitspapier nach einem der vorhergehenden Ansprüche, ferner eine Grundierungsschicht umfassend, die zwischen dem Substrat und der erkennbaren Schicht eingelegt ist.

11. Sicherheitspapier nach Anspruch 10, wobei die Grundierungsschicht ein wasserlösliches Harz umfasst.

12. Sicherheitspapier nach Anspruch 10 oder Anspruch 11, wobei die Dicke der Grundierungsschicht im Bereich von 0,1 µm bis 5 µm liegt.

13. Zusammensetzung zum Bilden einer erkennbaren Schicht, wobei die Zusammensetzung Folgendes umfasst: Metallpulver, eine siliciumhaltige Verbindung, ein wasserlösliches Bindemittelharz und Wasser.

14. Zusammensetzung nach Anspruch 13, wobei die Zusammensetzung ferner ein Dispergiermittel umfasst.

15. Verfahren zum Herstellen eines Sicherheitspapiers, wobei das Verfahren Folgendes umfasst:
Auftragen der Zusammensetzung nach einem der Ansprüche 13 und 14 auf mindestens einen Abschnitt mindestens einer Oberfläche eines Substrats und Trocknen der aufgetragenen Verbindung.

## Revendications

1. Papier de sécurité comprenant :
un substrat ; et
une couche détectable qui est attachée à au moins une partie d'au moins une surface du substrat,
dans lequel la couche détectable comprend de la poudre métallique, un composé contenant du silicium et une résine liante hydrosoluble.

2. Papier de sécurité selon la revendication 1, dans lequel le substrat est un papier qui est revêtu d'une résine, un papier qui n'est pas revêtu d'une résine ou un film de résine.

3. Papier de sécurité selon la revendication 1 ou la revendication 2, dans lequel la poudre métallique de la couche détectable est choisie dans le groupe constitué par le fer, le cobalt, le nickel, le manganèse et les associations de ceux-ci.

4. Papier de sécurité selon l'une quelconque des revendications précédentes, dans lequel la taille moyenne des particules de la poudre métallique est dans la plage de 0,1 µm à 100 µm.

5. Papier de sécurité selon l'une quelconque des revendications précédentes, dans lequel le composé contenant du silicium de la couche détectable est choisi dans le groupe constitué par les halogénosilanes, les alcoxysilanes, les aminosilanes, les agents de couplage silanes, les fluoroalkylsilanes, les oligomères de siloxane réactifs et les associations de ceux-ci.

6. Papier de sécurité selon l'une quelconque des revendications précédentes, dans lequel la résine liante hydrosoluble de la couche détectable est choisie dans le groupe constitué par un poly(alcool vinylique), une polyvinylpyrrolidone, un polyacrylate, un polyester, un latex et les associations de ceux-ci.

7. Papier de sécurité selon l'une quelconque des revendications précédentes, dans lequel la quantité de la poudre métallique dans la couche détectable est dans la plage de 1 % en poids à 10 % en poids sur la base de 100 % en poids du poids total de la couche détectable.

8. Papier de sécurité selon l'une quelconque des revendications précédentes, dans lequel la quantité du composé contenant du silicium dans la couche détectable est dans la plage de 1 % en poids à 50 % en poids sur la base de 100 % en poids du poids total de la couche détectable.

9. Papier de sécurité selon l'une quelconque des revendications précédentes, dans lequel l'épaisseur de la couche détectable est dans la plage de 1 µm à 10 µm.

10. Papier de sécurité selon l'une quelconque des revendications précédentes, comprenant en outre une sous-couche intercalée entre le substrat et la couche détectable.

11. Papier de sécurité selon la revendication 10, dans lequel la sous-couche comprend une résine hydrosoluble.

12. Papier de sécurité selon la revendication 10 ou la revendication 11, dans lequel l'épaisseur de la sous-couche est dans la plage de 0,1 µm à 5 µm.

13. Composition pour la formation d'une couche détectable, la composition comprenant : de la poudre métallique, un composé contenant du silicium, une résine liante hydrosoluble et de l'eau.

14. Composition selon la revendication 13, la composition comprenant en outre un agent dispersant.

15. Procédé de production d'un papier de sécurité, le procédé comprenant :
l'enduction de la composition selon l'une quelconque des revendications 13 et 14 sur au moins une partie d'au moins une surface d'un substrat ; et
le séchage de la composition enduite.
